

Patented May 17, 1927.

1,629,080

# UNITED STATES PATENT OFFICE.

FREDERICK LAIST AND FREDERICK F. FRICK, OF ANACONDA, MONTANA.

## CONCENTRATION OF MINERALS FROM ORES BY THE USE OF SULPHONES AS FLOTATION REAGENTS.

No Drawing.

Application filed April 13, 1926. Serial No. 101,793.

This invention relates to the concentration of minerals from ores by flotation.

The object of this invention is the provision of new and useful flotation reagents and processes of floating ores by their means.

We have discovered that the sulphones, in general, are effective flotation reagents. The sulphones are organic sulphur compounds of the general type represented by the formula



in which R and R' stand for organic radicals and O stands for oxygen. We have found that it makes little difference what the nature of the organic radicals R and R' is. R and R' in the above formula may stand for hydrocarbon radicals, such as the alkyl, aryl and aralkyl groups, as well as derivatives and homologues of the same. Typical sulphones, which are suitable for the purposes of this invention, are diphenyl sulphone,  $(\text{C}_6\text{H}_5)_2\text{SO}_2$ , and butyl sulphone,  $(\text{C}_4\text{H}_9)_2\text{SO}_2$ . We may also use mixed sulphones such as alkyl-aryl, alkyl-aralkyl and aryl-aralkyl sulphones.

In using the compounds of this invention as flotation reagents, they may be added to the ore to be floated in any suitable manner or place and at any stage prior to flotation or during flotation. They may be added to the grinding mill, to the pulp just before flotation or during flotation. These reagents may be used alone or combined with other reagents generally used in the flotation art, such as, for example, frothing reagents and agents for stabilizing the froth. They may also be used in combination with other flotation reagents.

In general, pine oil is used to advantage as a frother. Other oils, such as tar oils, may be used to stabilize the froth and aid in the recovery of the minerals.

These reagents may be used with ores generally; they may be found to work better with some ores in an acid circuit; with others in a neutral circuit, and in the case of still others in a circuit made alkaline with soda ash or burned lime.

Commercial or impure forms or solutions of these reagents may be used. They may be used in varying quantities. A quarter or even a tenth of a pound per ton of ore may prove effective in the case of some ores. In

others, a pound per ton of ore may be required.

The flotation pulp, containing a sulphone, is subjected to agitation and aeration in standard flotation machines. The following table is given, by way of illustration, to show the results when using normal butyl sulphone. It is to be understood that our invention is not limited to this specific reagent nor to the specific manner of its application recited in this example.

### *N-butyl sulphone on copper ore.*

Two tests are given, the first a test using sulphuric acid and pine oil, and the second, sulphuric acid, pine oil and n-butyl sulphone. The test conditions were identical except for the use of n-butyl sulphone in the second test.

|                          | Control test. | N-butyl sulphone test. |
|--------------------------|---------------|------------------------|
| Feed: % Cu               | 1.55          | 1.45                   |
| Concentrate: % Cu        | 2.63          | 7.75                   |
| Middling: % Cu           | 3.52          | 2.53                   |
| Tailing: % Cu            | 1.27          | .13                    |
| Reagents: #/ton feed:    |               |                        |
| Sulphuric acid           | 15.           | 15.                    |
| Steam distilled pine oil | 1.            | 1.                     |
| N-butyl-sulphone         |               | 1.                     |

The pine oil was used as a frothing reagent.

The effectiveness of this reagent is fully shown by the above table. The percentage of copper recovered was 92.9%.

We claim:

1. A process of concentrating ores by froth flotation, which comprises subjecting to a flotation operation a mixture of the ore containing a sulphone in a quantity effective for flotation.

2. A process of concentrating ores by froth flotation, which comprises subjecting to a flotation operation a mixture of the ore containing an organic sulphur compound of the general type



in which R and R' stand for hydrocarbon radicals or derivatives or homologues of the same, and O stands for oxygen in a quantity effective for flotation.

3. A process of concentrating ores by froth flotation, which comprises adding a

sulphone to the ground ore in a quantity effective for flotation and subjecting the mixture to a flotation operation.

4. A process of concentrating ores by froth flotation, which comprises adding to the ground ore an organic sulphur compound of the general type,



10 in which R and R' stand for hydrocarbon radicals or derivatives or homologues of the same, and O stands for oxygen, in a quantity effective for flotation and subjecting the mixture to a flotation operation.

15 5. A process of concentrating ores by froth flotation, which comprises adding to the ground ore an organic sulphur compound of the general type



in which R and R' may be alkyl, aryl or

aralkyl groups, and in which O stands for oxygen, in a quantity effective for flotation and subjecting the mixture to a flotation 25 operation.

6. The process of concentrating ores by froth flotation, which comprises adding to the ground ore an organic sulphur compound of the general type



30 in which both R and R' stand for alkyl groups and O stands for oxygen, in a quantity effective for flotation and subjecting the mixture to a flotation operation.

7. A process of concentrating ores by flotation, which comprises adding n-butyl sulphone to the ground ore and subjecting 40 the mixture to a froth flotation operation.

In testimony whereof, we affix our signatures.

FREDERICK LAIST.  
FREDERICK F. FRICK.